

## UNITED STATES PATENT OFFICE

ARMAN E. BECKER, OF ELIZABETH, NEW JERSEY, ASSIGNOR TO STANDARD OIL DEVELOPMENT COMPANY, A CORPORATION OF DELAWARE

## METHOD OF LUBRICATING TEXTILE MACHINERY

No Drawing.

Application filed September 20, 1926. Serial No. 136,721.

This invention relates to improvements in the lubrication of bearings and other moving parts of machines used in the fabrication of textiles. As is well known, it is practically impossible to prevent soiling of the textile product by the oil or grease used on the machines. Heretofore, difficulty has been met in securing a lubricating material which has satisfactory lubricating qualities and is also readily washed out of the textile product.

In accordance with the present invention, textile machines and their appurtenances are lubricated with a viscous hydrocarbon oil containing a small percentage of water-soluble soap. I prefer to use a petroleum oil of about 50 to 250 seconds Saybolt viscosity at 100° F., highly purified by treatment with sulphuric acid or contact with fuller's earth or the like or by any other methods known to the petroleum industry and containing about 0.15% to 1.5% by weight of an alkali metal soap of one or more of the higher fatty acids; for example, sodium oleate or sodium stearate, or mixtures of the same. For spindle lubrication, oils of 50 to 100 seconds Saybolt viscosity are most suitable, while for motor bearings and the like 75 to 250 viscosity at 100° F., or even higher, is desirable. The quantity of soap in oil for either purpose is generally between .15 and .20%.

The composition may be prepared in any suitable way, examples of which are described in applicant's Patent No. 1,628,646, patented May 17, 1927. In one process for making the composition, a mixture of viscous petroleum oil and the proper percentage of oleic acid is brought up to a temperature of about 180° F., with agitation. Then the calculated amount of a 10-25% aqueous solution of sodium hydroxid, required to substantially neutralize the oleic acid, is added. Agitation and heat are continued until the composition has reached a temperature of not less than 350° F. The composition is then rapidly cooled by passing it through an elongated cooling coil having many bends.

As mentioned above, highly purified oils are generally most desirable, because they do not become appreciably discolored on standing, nor impart objectionable coloration to

the fibers, nor have any disagreeable odor. The so-called "white oils" are particularly well adapted for this purpose. White oils are highly purified heavy petroleum oils, corresponding more or less closely to petro- 55 latum liquidum, U. S. P. However, the present method is not limited to the use of such oils. For example, oils of the ordinary lubricating grade may be used, especially in cases where some coloration is not objectionable. 60

The lubricants described above are applied to the bearings and other parts in the usual manner.

Various changes and alternative procedures may be adopted within the scope of 65 the appended claims, in which it is my intention to claim all novelty inherent in the invention as broadly as the prior art permits.

I claim:

1. In the lubrication of textile machine bearings and other moving parts from which the lubricant may come into contact with the textile product, the improvement that comprises supplying as a lubricant a petroleum oil to which has been added a small quantity of water-soluble alkali metal soap. 70

2. Process according to claim 1, in which a petroleum white oil is used.

3. Process according to claim 1, in which about 0.15 to 0.20% of an alkali metal soap is used. 80

4. Process according to claim 1, in which a substantial quantity of a water-soluble alkali metal soap, not exceeding 1.5% by weight of the lubricant is used. 85

5. In the lubrication of textile machine bearings and other moving parts from which the lubricant may come into contact with the textile product, the improvement that comprises supplying as a lubricant a petroleum oil having a viscosity of about 50 to 250 seconds Saybolt at 100° F., to which has been added about 0.15 to 1.5% of a water-soluble alkali metal soap. 90

6. Process according to claim 5, in which the soap used is sodium oleate. 95

ARMAN E. BECKER.